# EUROPEAN PATENT SPECIFICATION

(11) **EP 0 411 760 B1**
(45) Date of publication and mention of the grant of the patent: **08.11.1995**
(21) Application number: 90306895.5
(22) Date of filing: 31.07.1990
(51) Int. Cl.: G03C 5/38

(54) **Photographic processing**
Photographische Bearbeitung
Traitement photographique

(30) Priority: 04.08.1989 GB 8917920
(43) Date of publication of application: 06.02.1991
(73) Proprietor: EASTMAN KODAK COMPANY, Rochester, New York 14650-2201 (US); KODAK LIMITED, Hemel Hempstead Hertfordshire HP1 1JY (GB)
(72) Inventor: Fyson, John Richard, London E9 7AS (GB)
(74) Representative: Daley, Michael John

(56) References cited:
- WO-A-90/13060
- US-A- 2 174 494
- US-A- 2 515 122
- G. HAIST: "MODERN PHOTOGRAPHIC PROCESSING Volume 1", 1979, JOHN WILEY AND SONS, NEW YORK
- R.S. SCHULTZE: "SCIENCE AND APPLICATIONS OF PHOTOGRAPHY", 1955, ROYAL PHOTOGRAPHIC SOCIETY OF GB, LONDON; "Acceleration of the fixing process by active cations", pp 177-180

## Description

This invention relates to photographic processing and, in particular, to a method of fixing.

Photographic silver halide materials are employed to form images by first imagewise exposing the material, e.g. in camera, and then processing to form a visible image. The processing steps usually include (a) a development step in which the exposed areas of the material form a visible image and (b) a fixing step whereby the undeveloped silver halide is removed by treatment with a fixer solution which contains a silver halide solvent.

The most widely used fixer solutions are based on alkali metal or ammonium thiosulphates. Under certain conditions some colour couplers (as used in colour materials) can continue to couple in a thiosulphate fixer. Further, thiosulphate fixer solutions are unstable and can precipitate sulphur.

Our published International Application WO90/13060 proposes to use alkali metal sulphite solutions to remove silver chloride from photographic materials in acceptable processing times. However fixing is relatively slow in comparison with thiosulphate fixers. Reference is also made to our published International Applications WO90/13059 and WO90/13061.

"Science and Applications of Photography" (Ed. R.S. Schultze), 1955, pp. 177-180, discloses the use of active cations derived from piperidine or pyridine as fix-accelerators in hypo fixing solutions. "Modern Photographic Processing", (Grant Haist), Vol. 1, 1979, pp. 598-599, discloses the use of sodium sulphite as a fixing agent.

In accordance with the present invention there is provided a fixing method of removing silver halide, especially silver chloride, from a photographic material during processing which comprises treatment with a hypo-free aqueous solution containing an alkali metal sulphite, characterised in that the solution has a pH in the region of 8 and also contains a water soluble quaternary nitrogen compound.

The quaternary nitrogen compound should have a relatively strong conjugate base so that, at the pH prevailing in a fixing solution, in the region of 8, it is protonated and cationic. One suitable compound is ethylenediammonium sulphate$\text{H₃} {\text{N}}^{+} \text{-C-C-} {\text{N}}^{+} {\text{H₃ . SO}}_{\text{4}}^{\text{2-}}$

We have found that particularly in sodium and potassium sulphite fixing solutions incorporating these quarternary ammonium compounds the fixing rate is surprisingly enhanced.

The following example illustrates the present invention and the accompanying drawing is a graph of residual silver against fixing time.

### EXAMPLE 1

A coloured paper coated with silver was produced from silver chloride. The following are the silver coating weights: 0.1076 mg/dm² the red and green sensitive layers and 0.4306 mg/dm² in the blue sensitive layer layer, giving a total silver laydown of 0.6459 mg/dm².

Sample strips of this coated paper were swollen in a 25g/1 potassium carbonate buffer pH 10.1 to simulate a developer. The strips were then plunged into a fixing solution in accordance with the invention (25°C) and processed for varying times. The strips were then washed for 2 minutes in water and treated with a 5g/1 sodium sulphide solution to reveal any residual silver chloride as silver sulphide. The strips were then washed for a further 2 minutes, then hung up to dry. The blue reflection density of each strip was measured. It was found that the maximum density for the unfixed sample was 0.30 and for a totally fixed sample, 0.05. Atomic adsorption measurements of the silver showed that there was a good linear correlation between blue reflection density and residual silver. From the density measurements, it was therefore possible to estimate the residual silver in the paper.

Three fixing solutions were made up and the pH of all of them was adjusted to 8.0 ± 0.1, see the table below. The results are shown in the drawing. The gradient of the best fit straight line through the experimental points is taken as a measure of the relative fixing rate of the materials and is included in the table below.

It can be seen that the fixing rate by the solution containing the quaternary salt and the sulphite (Fix 3) is three times greater than the sum of the two rates in the fixer containing the separate components, indicating that the two are working synergistically.

The fixing action of the ethylenediammonium sulphate is probably by the free base ethylenediamine which is present at small concentrations at pH8.0.

A Similar experiment was carried out with n-methyl pyridinium chloride. This substance had no fixing action in itself. A 20g/1 sulphite fixing solution containing 5g/1 of this salt had a relative fixing rate of 0.27 calculated on a similar basis to the above.

The fixing method and solution as described are useful with photographic silver halide elements known in the photographic art. A description of illustrative examples of such photographic materials is found in, for instance, Research Disclosure, Item No. 17,463 Vol. 176, pages 22 - 31 (December 1978).

## Claims

1. A fixing method of removing silver halide from a photographic material during processing such method comprising treatment with a hypo-free aqueous solution containing an alkali metal sulphite, characterised in that the solution has a pH in the region of 8 and also contains a water soluble quaternary nitrogen compound.

2. A method as claimed in Claim 1 wherein the silver halide is silver chloride.

3. A method as claimed in either Claim 1 or Claim 2 wherein the the quaternary compound has a strong conjugate base.

4. A method as claimed in either Claim 1 or Claim 2 wherein the quaternary compound is ethylenediammonium sulphate.

5. A method as claimed in any preceding claims characterised in that the fixing solution has a pH of 8.0 ± 0.1.

6. A hypo-free fixing solution comprising an alkali metal sulphite, characterised in that said solution has a pH in the region of 8 and also contains a water soluble quaternary nitrogen compound.

## Patentansprüche

1. Fixierverfahren zur Entfernung von Silberhalogenid von einem photographischen Material während der Bearbeitung, wobei das Verfahren die Behandlung mit einer hypofreien wäßrigen Lösung, die ein Alkalimetallsulfit enthält, umfaßt und
dadurch **gekennzeichnet** ist, daß die Lösung einen pH-Wert im Bereich von 8 hat und außerdem eine wasserlösliche quartäre Stickstoffverbindung enthält.

2. Verfahren nach Anspruch 1, wobei das Silberhalogenid Silberchlorid ist.

3. Verfahren nach Anspruch 1 oder 2, wobei die quartäre Verbindung eine starke konjugierte Base hat.

4. Verfahren nach Anspruch 1 oder 2, wobei die quartäre Verbindung Ethylendiammoniumsulfat ist.

5. Verfahren nach einem der vorhergehenden Ansprüche, dadurch **gekennzeichnet**, daß die Fixierlösung einen pH-Wert von 8,0 ± 0,1 hat.

6. Hypofreie Fixierlösung, die ein Alkalimetallsulfit enthält,
dadurch **gekennzeichnet**, daß die Lösung einen pH-Wert im Bereich von 8 hat und außerdem eine wasserlösliche quartäre Stickstoffverbindung enthält.

## Revendications

1. Procédé de fixage par enlèvement d'halogénure d'argent d'un matériau photographique pendant le traitement, ce procédé comprenant une solution aqueuse sans hypo contenant un sulphite des métaux alcalins, caractérisé en ce que la solution a un pH dans la plage de 8 et contient également un composé d'azote quaternaire hydrosoluble.

2. Procédé selon la revendication 1, dans lequel l'halogénure d'argent est un chlorure d'argent.

3. Procédé selon l'une quelconque des revendications 1 ou 2, dans lequel le composé quaternaire possède une base de conjugué forte.

4. Procédé selon l'une quelconque des revendications 1 ou 2, dans lequel le composé quaternaire est un éthylène diammonium sulfate.

5. Procédé selon l'une quelconque des revendications précédentes, caractérisé en ce que la solution de fixage a un pH de 8,0 ± 0,1.

6. Solution de fixage sans hypo comprenant un sulphite des métaux alcalins caractérisé en ce que la solution présente un pH dans la plage de 8 et contient également un composé d'azote quaternaire hydrosoluble.
